

J. A. E. CRISWELL,  
MATCH.  
APPLICATION FILED JUNE 13, 1906.

988,251.

Patented Mar. 28, 1911.



Witnesses  
William F. Linn  
O. H. Stanley

Inventor  
J. A. Criswell

# UNITED STATES PATENT OFFICE.

JAMES A. EKIN CRISWELL, OF NEW YORK, N. Y.

## MATCH.

988,251.

Specification of Letters Patent. Patented Mar. 28, 1911.

Application filed June 13, 1905. Serial No. 265,095.

*To all whom it may concern:*

Be it known that I, JAMES A. EKIN CRISWELL, of New York, county of Kings, and State of New York, have invented certain 5 new and useful Improvements in Matches, of which the following is a full, clear, and exact description.

This invention relates more particularly to matches made from materials which have 10 been reduced to a plastic condition.

The main object of the invention is to provide a composite match having an inner body and an outer surface of paper-making material of different density, whereby the 15 match stem or body may be strengthened and at the same time avoid the liability of preventing the body from properly absorbing the paraffin or other flame-carrying medium.

20 A further object of the invention is to provide matches which may be made wholly or in part of cheap materials on each of which may be placed suitable advertising matter.

25 The invention will be hereinafter more particularly described with reference to the accompanying drawings, which form a part of this specification, and will then be pointed out in the claim at the end of the description.

30 In the drawings, Figure 1 is a perspective view of one form of match embodying the invention. Fig. 2 is an enlarged transverse section taken on the line II—II of Fig. 3. Fig. 3 is a longitudinal section taken on the 35 line III—III of Fig. 2. Fig. 4 is an enlarged transverse section of a slightly different form of match body or stem.

40 The match body or stem 10 has an inner body or core 11, an outer casing or cover 12, and an igniting head of any suitable material 13. The entire match body is made of paper-making pulp which includes any or all of the materials of which paper may be 45 made. The inner body 11 is preferably made of very cheap material, or materials that ordinarily go to waste, such as old newspapers, scraps, refuse, and the like which is reduced to a pulp or pulpy condition according to 50 the usual methods employed in the manufacture of paper. These materials may be united with plaster of Paris, copperas or the like to assist in hardening the same, and may

be compressed sufficiently to form rods or wires of said material. Around the body 11 55 is formed a coating or cover 12 of paper-making pulp which may be of better material, such as a combination of the other materials with sulfite pulp, so that the match body when completed will be sufficiently 60 strong and of an attractive appearance. The cover or casing 12 may be formed in a web, but not compressed to the full extent as in making complete marketable paper, or if made into paper it may be of a soft character and may be applied in a wet state. When the cover 12 is formed around the body 11 and the whole suitably compressed by running between fluted or grooved rollers, or otherwise, the proper density of the inner 70 body and outer cover is obtained, and the two parts thus united and compressed together form a substantially homogeneous match body with the fibers of one working into and united with fibers of the other. 75

If desired glutinous or resinous substances may be added to assist in uniting the inner body and outer covering together; and the inner body may be made of old printed newspapers reduced to a pulp and united 80 with any suitable hardening material, as for example, plaster of Paris, and the body of the matches may be run through paraffin, stearin, wax and the like to form a coating 85 14, as shown in Fig. 4.

It will be seen that matches made according to the method described will be homogeneous in character, strong and uniform in character, and attractive in appearance.

It will be understood that various materials may be added to assist in the burning, and in various proportions and combinations, and that paraffin or similar material may be added at any stage of the manufacture. Materials such as saltpeter, sulfur, 95 rosin and the like may be added to assist in making the match bodies burn more freely, and any of the materials may be impregnated with phosphate of ammonia, phosphoric acid, or other chemicals to prevent 100 the body from retaining the fire after the flame is blown out, and when materials of this character are used.

The matches may be of any desired shape to make them distinctive, and on each match 105 body or stem may be placed suitable adver-

tising matter for advertising various articles of manufacture.

Having thus described my invention, what I claim as new and desire to secure by Letters Patent, is—

A match having its stem made of plastic material comprising a relatively hard inner

body of paper-making pulp, a coating therefor of paper-making pulp of less density and an igniting head on the body.

J. A. EKIN CRISWELL.

Witnesses:

M. TURNER,  
A. CLEMENTS.